

Jan. 10, 1967

D. J. RANSOM ET AL

3,297,416

CONTROL OF HYDROGEN EMBRITTLEMENT

Filed April 24, 1964

FIG. 1



FIG. 2



FIG. 3



INVENTORS  
DONALD J. RANSOM  
ELI SIMON  
MYRON LEVINE

By *George Sullivan*  
Agent

3,297,416

**CONTROL OF HYDROGEN EMBRITTLEMENT**  
Donald J. Ransom, Sylmar, and Eli Simon and Myron Levine, Los Angeles, Calif., assignors to Lockheed Aircraft Corporation, Burbank, Calif.Filed Apr. 24, 1964, Ser. No. 362,397  
14 Claims. (Cl. 29—195)

This invention pertains to the field of hydrogen embrittlement of a metal.

It is well-known that certain metals such as common 4340 steel are susceptible to so-called hydrogen embrittlement. A complete understanding of this hydrogen embrittlement problem is unnecessary to an understanding of the present invention. Briefly, however, this problem concerns the fact that when a small quantity of nascent hydrogen is "available" at the surface of a metal susceptible to hydrogen embrittlement this hydrogen will tend to enter the structure of the metal, causing a decrease to the load sustaining capacity of the metal itself.

It is considered that the most effective means for controlling corrosion at the surface of a metal susceptible to hydrogen embrittlement is through the use of a protective metal coating. Thus, for example, with the 4340 high-strength steel referred to above it is known to protect against corrosion by locating upon a surface of the metal a protective coating of cadmium. For various high temperature uses a combination of nickel and cadmium may be employed instead of cadmium. Such metal coatings are normally at least .0003 inch thick and are frequently from about .0004 to .0005 inch thick. Under circumstances as hereinafter explained hydrogen embrittlement may occur in the presence of such metal coatings.

Protective metal coatings of this type may be applied to a metal surface in several manners. Thus, for example, a cadmium coating can be applied to a surface by a known vacuum deposition type of process. In general the coatings produced in this manner tend to be somewhat porous also with them adhesion can be a problem. Protective coatings of cadmium can also be applied by electroplating processes as are disclosed in the Simon et al. Patent No. 2,892,761 and the Hamilton et al. Patent No. 3,014,852 assigned to the Lockheed Aircraft Corp. The entire contents of these patents are incorporated herein by reference for the purpose of amplifying upon and supplementing the contents of this specification.

An object of the present invention is to provide new and improved procedures for preventing and/or controlling hydrogen embrittlement. A related object of this invention is to provide new and improved surface structures for use in combatting the problem of hydrogen embrittlement. Other objects of the present invention are to provide methods and structures as indicated which are comparatively inexpensive, effective and easy to carry out and create, respectively.

These and further objects of this invention as well as many advantages of it will be more fully apparent from a detailed consideration of the remainder of this specification, the appended claims and the accompanying drawing in which:

FIGURE 1 is an enlarged cross-sectional diagrammatic view indicating a surface structure in accordance with this invention;

FIGURE 2 is a view similar to FIGURE 1 of a modified surface structure of this invention; and

FIGURE 3 is a view similar to FIGURE 1 of a further modified surface structure of this invention.

It will be apparent from a consideration of the drawing and the remainder of this specification that none of the figures of the drawing are intended to represent any precise structure, but that these figures are primarily

intended for explanatory purposes. From a consideration of the drawing and the remainder of this specification it will be obvious to those skilled in the hydrogen embrittlement field that the present invention can be utilized in a number of different manners falling within the scope of the appended claims.

As an aid to understanding this invention it can be stated in essentially summary form that it concerns control of hydrogen embrittlement upon a metal member which is susceptible to such embrittlement through the location upon such a member of one or more oxidizing agents which: (1) are inert with respect to materials in contact with such an agent or agents; (2) are stable under the ambient conditions to which the metal member may be subjected; and (3) are capable of reacting with any nascent hydrogen liberated at the surface of the member in order to protect the metal member from hydrogen embrittlement by combining with such hydrogen. Preferably the metal member is coated with a protective metal coating serving to protect against corrosion. The oxidizing agent or agents used can be located upon such a protective coating. If desired a surface structure of this type can be referred to as an "article of manufacture."

This invention is best more fully explained by referring directly to FIGURE 1 of the drawing. Here there is shown a metal member such as a 4340 high-strength steel member 10 having a surface 12 which is covered with a cadmium protective coating 14. This coating 14 may be applied to the surface 12 by vacuum deposition techniques or as described in either of the aforesaid patents. In accordance with this invention the exposed surface 16 of the coating 14 is covered with a coating or layer 18 containing one or more oxidizing agents.

The purpose of this layer 18 and its function can be related to what may occur at the surface 12 in the absence of the layer 18. The metal cadmium is of anodic nature with respect to steel. In the presence of humid or especially a humid salt containing atmosphere there is a tendency for a reaction to take place between those two metals. As a consequence of this reaction it is considered that hydrogen is to a degree liberated, and that this hydrogen as a result of the lower hydrogen over-voltage on steel as compared to cadmium will tend to enter the steel, causing hydrogen embrittlement. It is not considered necessary to set forth herein the exact mechanism by which such hydrogen enters the structure of the steel and acts so as to lower its strength.

The layer 18 is located directly against the coating 14 so as to be as closely adjacent to the surface 12 as reasonably possible. Because of the somewhat porous, hydrogen permeable character of the layer 18 any hydrogen liberated as a result of reactions as are indicated in preceding paragraphs will react with an oxidizing agent disposed within this layer 18 to a sufficient degree to provide significant protection against hydrogen embrittlement. Such reaction will have the effect of immobilizing the hydrogen, preventing it entering through the surface 12 so as to cause embrittlement.

The particular layer 18 illustrated in FIGURE 1 of the drawing consists of a mixture of at least one oxidizing agent disposed within a small amount of an inert fluid or viscous type of composition serving as a movable binder to hold the oxidizing agent in place. Virtually any inert or substantially inert carrier type of vehicle can be employed for the purpose of holding one or more oxidizing agents in place so as to form the layer 18. Thus, it is possible to utilize various conventional mineral and silicone greases and oils, fluid plasticizers such as are commonly employed in the plastic field, petroleum jelly fractions or the like. If desired one or more volatile solvents can be initially present with such vehicles for the purpose

of facilitating the application of a composition as herein described.

The oxidizing agent or agents used with this invention should be inert both with respect to the member 10 and to the coating 14. Also, any such oxidizing agent or agents should be stable at the ambient conditions to which the member 10 will be subjected during its use. Obviously any such oxidizing agent or agents should be capable of reaction with nascent hydrogen so as to immobilize it in order to prevent such hydrogen from entering the metal surface.

A large number of different oxidizing agents meet these criteria. Presently preferred inorganic oxidizing agents belong to the class of known perborate and nitrate oxidizing agents such as sodium perborate, sodium nitrate and related alkali metal and alkaline earth compounds, although other inorganic oxidizing agents such as various permanganates, manganese dioxide, lead dioxide and the like can be used depending upon the temperature and the degree of stress imposed on the high strength steel.

A number of different organic oxidizing agents can also be employed at various temperatures, among such peroxides are those listed in Table 4 on page 78 of the text *Vinyl and Related Polymers* by Schildknecht published by John Wiley & Sons, Inc., New York, New York, 1952. This list is incorporated herein by reference in the interest of brevity. This list specifies various temperature operating ranges at which the peroxides listed can be used. Other organic oxidizing agents capable of being used with this invention at different temperature ranges are various compounds capable of being used for photographic development and related purposes. Thus, for example, quinone, anthraquinone, benzyl, naphthaquinone, phenanthraquinone, quinonimine, various vat dyes and the like can be employed at temperatures at which these compounds are stable in order to achieve advantages of this invention.

It is presently preferred to create a layer 18 by the simple expedient of mixing the ingredients present in this layer together and then to wipe or smear this mixture on a surface. Following these operations it is normally preferred to reduce the thickness of the layer 18 to roughly the thickness of a "wiped" Vaseline film by wiping with a cloth or the like. In general the relative proportions of the ingredients within the layer 18 are not "critical" so long as this layer 18 contains as much oxidizing material as conveniently possible. In general the higher the proportion of the oxidizing agent or agents present the more effective the results achieved. What is important is the presence and availability of an oxidizing agent to the surface 12.

As an example of how to create a layer such as the layer 18 acceptable results can be achieved by covering cadmium coated 4340 steel surfaces with a layer of any of the following mixtures, and then wiping these layers with a cloth so as to leave only a thin film:

*Composition 1.*—50 parts by weight benzoyl peroxide; 50 parts by weight tricresyl phosphate; 10 parts by weight toluene.

*Composition 2.*—50 parts by weight benzoyl peroxide; 50 parts by weight of a conventionally known inert silicone oil such as the silicone oil produced by the Dow Chemical Corporation of Midland, Michigan, and sold under the trade name designation DC-200.

*Composition 3.*—20 parts by weight sodium nitrate and 80 parts by weight of the inert silicone oil specified in the preceding composition 2 (in this case the ingredients should be milled together so as to obtain an intimate mixture).

In FIGURE 2 of the drawing there is shown a metal member 20 corresponding to the member 10 having a surface 22 holding a relatively porous cadmium coating 24. This coating 24 can be applied to this surface 22 by known vacuum deposition techniques so as to be of a porous character. In the drawing this coating 24 has

been hatched so as to simulate to as great a degree as possible its porous character. The pores within this coating 24 are filled with at least one oxidizing agent 26 as described in the preceding.

The pores may be filled with an organic oxidizing agent as described in the preceding by merely forming a solvent solution of such an agent such as a saturated solution of benzoyl peroxide in benzene and then impregnating the coating 24 in the known manner in which capacitors are vacuum impregnated with a dielectric material. After this is done the solvent is of course removed by vaporization. Such impregnation may be repeated several times in order to assure the presence of as much oxidizing agent in the pores as reasonably possible. In the same manner an aqueous solution of sodium nitrate may be applied to a porous cadmium surface 24 and the water removed as soon as possible by vaporization, leaving sodium nitrate within the pores of the coating 24.

In FIGURE 3 of the drawing there is shown another metal member 30 corresponding to the member 10 previously described which has a surface 32 covered by an adherent coating 34 of a cadmium-nickel alloy type composition serving to provide protection against corrosion. The normally exposed surface 36 of the coating 34 is covered with an adherent layer 38 of a paint or lacquer-like character containing one or more oxidizing agents capable of being used with this invention, and conventional inert ingredients serving as a permanent binder. The particular construction shown in FIGURE 3 is considered to be particularly desirable for use where the member 30 is subjected to relatively high temperatures.

The layer 38 may consist of one or more oxidizing agents as indicated in the preceding discussion dispersed within virtually any type of a paint or lacquer-like binder composition. Such compositions are, of course, much more stable and resistant to removal than compositions such as are capable of being used in creating the layer 18 previously described. If an inorganic oxidizing agent or if inorganic oxidizing agents are to be employed in the coating 38 such material or materials can be handled in substantially the same manner as any fillers or pigments within paint or lacquers, and such paints or lacquers can be either of a type which cure by virtue of the presence of one or more catalysts within them promoting the reaction of a polymerized or partially polymerized ingredients or of a solvent-release non-curing type. The organic oxidizing agents used in forming a layer such as the layer 38 preferably are only employed with so-called "non-curing" type paint or lacquer compositions in order to avoid any possibility of these compounds entering into reactions with these compositions. The amount of one or more oxidizing agents used in any of these types of compositions should preferably correspond to the amount of filler and pigment conventionally used in a paint or lacquer.

As an example as to how a coating such as the coating 38 may be created, it may be merely created from a lacquer type of composition containing: 15 parts by weight of a well known vinyl chloride-vinyl acetate-vinyl alcohol co-polymer such as is sold under the trade name designation VAGH by the Carbide and Carbon Corporation, New York, New York; 3 parts by weight tricresyl phosphate; 5 parts by weight benzoyl peroxide; 30 parts by weight methyl isobutyl ketone; and 30 parts by weight toluene. This composition can be applied and dried in the same manner as any conventional lacquer. If desired one half of the benzoyl peroxide in this composition can be replaced by lauroyl peroxide.

An inorganic type paint type of composition capable of being used in creating a layer such as the layer 38 can be manufactured from: 20 grams sodium nitrate; 22.8 grams raw linseed oil; 3.6 grams turpentine; and 0.6 gram Japan drier in the same manner in which a paint is manufactured. This composition can be used in substantially the same manner as any conventional paint.

If desired, this composition can be modified so as to substitute for a part of the sodium nitrate, such as one half of the sodium nitrate, an equivalent weight of sodium perborate.

From a careful consideration of this specification those skilled in the field of hydrogen embrittlement will realize that the means herein described for controlling such embrittlement are comparatively inexpensive, simple to use or apply and effective. Such individuals will further realize that an important aspect of the present invention lies not in precise proportions of an oxidizing agent used, but in the presence of such an oxidizing agent adjacent to a surface susceptible to hydrogen embrittlement when this agent is needed in order to react with hydrogen. Because of the nature of this invention it is to be considered as being limited solely by the appended claims forming a part of this disclosure.

We claim:

1. An article of manufacture which comprises: a high-strength steel member of a type susceptible to 20 hydrogen embrittlement, said member having a surface; a porous, hydrogen-permeable metal coating covering said surface; and an oxidant located adjacent to said coating, said oxidant 25 being chemically inert with respect to said steel member, being stable under the ambient conditions to which said steel member may be subjected and being capable of reaction with nascent hydrogen at the surface of said steel member in order to prevent 30 hydrogen from entering said surface.
2. An article of manufacture which comprises: a metal member susceptible of hydrogen embrittlement, said member having a surface; a porous, hydrogen-permeable metal coating located 35 against said surface; and an oxidizing agent selected from the group comprising alkali metal perborates, alkaline earth perborates, alkali metal nitrates, alkaline earth nitrates, permanganates, manganese dioxide, lead dioxide, benzoyl peroxide, quinone, anthraquinone, benzil, naphthaquinone, phenanthraquinone, and quinonimine, located adjacent to said surface, said oxidizing agent being capable of reacting with any hydrogen liberated as a result of anodic reaction between said metal 40 member and said metal coating in order to protect said metal member from hydrogen embrittlement resulting from such liberation of hydrogen.
3. An article of manufacture as defined in claim 2 wherein said metal coating is selected from the group 45 comprising cadmium, and nickel-cadmium alloy.
4. An article of manufacture as defined in claim 2 including an organic viscous liquid binder carrying said oxidizing agent.
5. An article of manufacture as defined in claim 3 55 wherein said binder is selected from the group comprising mineral oil, mineral grease, fluid plasticizers, petroleum jelly fractions, silicone oil, and silicone grease.
6. In the combination of a metal member susceptible to hydrogen embrittlement having a surface covered with 60 a porous protective metal coating serving to protect said surface against corrosion, the improvement which comprises: an adherent layer located adjacent to said surface in contact with said protective metal coating, said adherent layer comprising the combination of: 65 a co-polymer vehicle comprising;

vinyl chloride-vinyl acetate-vinyl alcohol; an adherent comprising; a mixture of tricresyl phosphate and benzoyl peroxide; and a solvent comprising; a mixture of methyl isobutyl ketone and toluene; said layer being reactive with nascent hydrogen at the surface of said metal member in order to protect said metal member from hydrogen embrittlement.

7. A method of controlling hydrogen embrittlement at the surface of a metal member which is susceptible to such embrittlement which comprises the step of locating adjacent to the surface of said metal member an oxidizing agent which is substantially chemically inert with respect to said metal member, which is stable under ambient conditions and which is capable of reacting with any nascent hydrogen at the surface of said metal member and thereby protect said metal member from hydrogen embrittlement by combining with such hydrogen.

8. A method as defined in claim 7 wherein said metal member is a steel member.

9. A method as defined in claim 8 wherein said metal member is coated with an adherent metal coating containing cadmium, said metal coating serving to protect said metal member against corrosion.

10. A method as defined in claim 9 wherein said metal coating is porous and wherein said oxidizing agent is located within the pores of said metal coating.

11. A method as defined in claim 8 wherein said oxidizing agent is located upon the surface of said metal coating and is secured to the surface of said metal member by a viscous liquid binder.

12. In the combination defined in claim 6 wherein said adherent includes:

lauroyl peroxide.

13. In the combination of a metal member susceptible to hydrogen embrittlement having a surface covered with a porous protective metal coating serving to protect said surface against corrosion, the improvement which comprises:

an adherent layer located adjacent said surface in contact with said protective metal coating, said layer comprising:

a vehicle mixture of linseed oil, turpentine, and Japan dryer; and, an adherent comprising:

sodium nitrate, said layer being reactive with nascent hydrogen at the surface of said metal member and thereby protect said member against hydrogen embrittlement.

14. In the combination defined in claim 13 wherein said adherent includes:

sodium perborate.

#### References Cited by the Examiner

##### UNITED STATES PATENTS

|           |        |              |       |        |
|-----------|--------|--------------|-------|--------|
| 1,673,271 | 6/1928 | Stewart      | ----- | 148-14 |
| 2,892,761 | 6/1959 | Simon et al. | ----- | 204-50 |
| 3,178,321 | 4/1965 | Satterfield  | ----- | 148-14 |
| 3,181,978 | 5/1965 | Weiner       | ----- | 148-14 |

HYLAND BIZOT, Primary Examiner.

DAVID L. RECK, Examiner.

R. O. DEAN, Assistant Examiner.